

## UNITED STATES PATENT OFFICE

2,509,918

## METHOD OF REMOVING NICKEL AND CO-BALT IMPURITIES FROM ZINC ELECTROLYTE SOLUTIONS

Dinsmore Laurence Griffith and Mavis Jean Rankin, Flin Flon, Manitoba, Canada, assignors to Hudson Bay Mining and Smelting Co., Limited, Winnipeg, Manitoba, Canada

No Drawing. Application March 5, 1946,  
Serial No. 652,246

4 Claims. (Cl. 23—125)

1

This invention relates to the removal of impurities present in zinc electrolyte solutions prior to the recovery of zinc therefrom by the electrolytic method, and it is directed particularly to the removal of cobalt and nickel from such solutions.

It is well known that impurities in the electrolyte cause great difficulty during the operation of plating by electrical methods, in some cases due to the impurity itself plating and so causing the deposit to be impure and of less value, and in other cases due to the impurity bringing about a lowered efficiency in the plating process. Consequently great pains are taken and much expense is incurred in removing the harmful impurities so far as possible.

It has for many years been known that purification of an electrolyte may be effected by the displacement of one metal from the solution by another higher in the electromotive series and that such a displacement may be aided by the presence of a metal low in the electromotive series. Thus it is common, after iron and other metals have been precipitated by treating an electrolyte with zinc oxide or roasted zinc ore or lime while air is blown through the solution, to treat it with zinc dust and to increase the purifying action of the zinc dust by coating it with finely divided copper. This copper is commonly formed by precipitating it from the solution to be purified by the zinc dust.

On the basis of the above generalization as to removal of one metal in solution by another metal higher in the electromotive series, and this removal being aided by the presence of a metal low in the electromotive series, one would expect that all of the impurities could be removed without serious difficulties. Experiments have shown, however, that certain elements such as cobalt and nickel, which should, from the position assigned to them in the electromotive series, easily be removed, are exceedingly difficult to precipitate, the difficulty becoming more pronounced as the quantity of the impurities present in the electrolyte becomes less. Thus, it has not been possible to remove more than a few milligrams per litre, say from about 15 down to about 10 milligrams per litre, of such impurities as cobalt and nickel, and much work has been done to determine methods of removing these and other impurities which are similarly difficult to precipitate.

It has been proposed to use arsenic with zinc dust and copper but we have found that zinc dust, copper and arsenic additions alone are of little, if any, value in removing impurities such

2

as cobalt and nickel and this is illustrated by the following experiment which was carried out with a sample of tankhouse electrolyte (electrolyte ready for electrolysis in the hydro-metallurgical process for winning zinc) having the following analysis:

|            |                      |           |
|------------|----------------------|-----------|
| Zinc       | grams per litre      | About 120 |
| Copper     | milligrams per litre | 0.4       |
| 10 Cadmium | do                   | 0.3       |
| Cobalt     | do                   | 16.0      |
| Arsenic    | do                   | 0.04      |
| Antimony   | do                   | 0.024     |

Zinc dust and copper were then added to this electrolyte, using the normal small amounts, namely, 5 grams per litre of zinc dust and 1.4 grams per litre of copper as copper sulphate. Then purification tests were run on samples of this electrolyte with additions of arsenic (as arsenic oxide dissolved in sodium hydroxide and water, and neutralized to methyl orange with sulphuric acid) as set forth below, the samples being agitated for one hour at 45° C. The analyses of the filtrates from these tests were as follows:

| Test | Extra Additions    | Analysis of treated solution in milligrams per litre |     |      |      |       |
|------|--------------------|------------------------------------------------------|-----|------|------|-------|
|      |                    | Cu                                                   | Cd  | Co   | As   | Sb    |
| 30   |                    |                                                      |     |      |      |       |
| A    | 50 mg./l. Arsenic  | 0.5                                                  | 0.2 | 11.0 | .5   | 0.022 |
| B    | 100 mg./l. Arsenic | 0.6                                                  | 0.2 | 12.0 | 1.5  | 0.026 |
| C    | 200 mg./l. Arsenic | 0.7                                                  | 0.2 | 12.6 | 8.0  | 0.024 |
| D    | 300 mg./l. Arsenic | 4.5                                                  | 0.3 | 12.9 | 20.0 | 0.028 |

We have discovered that surprisingly good results are obtained in the removal of impurities and particularly cobalt if small amounts of both silver and arsenic in the form of soluble compounds are present in addition to the normal small amounts of zinc dust and a soluble copper compound. The amount of silver to be added varies according to the concentration of impurities in the particular electrolyte to be purified and precise directions as to the addition required for a given degree of purification may, therefore, not be stated. However, tests made on samples of tankhouse electrolyte show that remarkably good results are obtained with as little as 100 milligrams per litre of silver and that about 500 milligrams per litre is usually sufficient to reduce cobalt and nickel present as impurities to very small amounts.

Thus 250 milligrams per litre of silver in the form of silver sulphate crystals with 150 milli-

grams per litre of arsenic made cobalt not detectable in a sample of tankhouse electrolyte of the following analysis:

Zinc ----- grams per litre About 120  
 Copper ----- milligrams per litre 0.4  
 Cadmium ----- do 0.9  
 Cobalt ----- do 16.5  
 Arsenic ----- do 0.02  
 Antimony ----- do 0.028

The additions of zinc dust and copper were as set forth above and, after agitation for one hour at 45° C., the analysis of the filtrate in milligrams per litre was as follows:

| Cu  | Cd  | Co               | As  | Sb    |
|-----|-----|------------------|-----|-------|
| 0.3 | 0.2 | ( <sup>1</sup> ) | 0.2 | 0.024 |

<sup>1</sup> Not detectable.

The addition of silver as well as zinc dust, copper and arsenic also lead to very good results in the removal of nickel. Thus 500 milligrams per litre of silver as silver sulphate and 175 milligrams per litre of arsenic in sulphuric acid solution together with zinc dust and copper, as set forth above, were added to a sample of tankhouse electrolyte of the following analysis:

Zinc ----- grams per litre 135 30  
 Cadmium ----- milligrams per litre 0.4  
 Antimony ----- do 0.02  
 Copper ----- do 0.5  
 Arsenic ----- do 0.02  
 Cobalt ----- do 23.6 35  
 Nickel ----- do 18.8

After agitation for one hour at 40° C., the analysis of the filtrate in milligrams per litre was:

|              | Milligrams per litre |
|--------------|----------------------|
| Nickel ----- | 1.8                  |
| Cobalt ----- | 1.2                  |

The considerable effect of the silver addition is apparent on comparing the above analyses with the following result of a corresponding test carried out on the same electrolyte without any addition of silver. The analysis was:

|              | Milligrams per litre |
|--------------|----------------------|
| Nickel ----- | 13.6                 |
| Cobalt ----- | 18.0                 |

Other tests carried out showed that bismuth, gold, iron, cadmium, mercury, chromium, molybdenum, phosphorus, gallium, tungsten, sulphur, tellurium, germanium, selenium, nickel, palladium and platinum are, amongst others, of no value along with zinc dust, copper and arsenic; indeed certain of these metals, as for example platinum, are very detrimental, since not only is cobalt not removed, but the solution is left high in copper and arsenic.

What we claim as our invention is:

1. A method of removing impurities from zinc electrolyte, comprising contacting the electrolyte with small amounts of zinc dust, in the presence of small amounts of soluble copper, arsenic and silver compounds.

2. A method of removing impurities from zinc electrolyte solutions, comprising contacting the electrolyte with small amounts of zinc dust, in the presence of small amounts of soluble copper and arsenic compounds and from about 100 to about 500 milligrams per litre of silver in the form of a soluble compound.

3. A method of removing impurities from zinc electrolyte solutions, comprising adding to the electrolyte small amounts of zinc dust, copper sulphate, a soluble arsenic compound and a soluble silver compound.

4. A method of removing impurities from zinc electrolyte solutions comprising adding to the electrolyte small amounts of zinc dust, copper sulphate, a soluble arsenic compound and from about 100 to 500 milligrams per litre of silver in the form of a soluble compound.

DINSMORE LAURENCE GRIFFITH.  
 MAVIS JEAN RANKIN.

#### REFERENCES CITED

The following references are of record in the file of this patent:

#### UNITED STATES PATENTS

| 45 | Number    | Name            | Date          |
|----|-----------|-----------------|---------------|
|    | 1,403,065 | Avery et al.    | Jan. 10, 1922 |
|    | 1,733,676 | Stevens et al.  | Oct. 29, 1929 |
|    | 2,396,569 | Griffith et al. | Mar. 12, 1946 |